

Dec. 15, 1942.

H. T. COSS ET AL

**2,305,516**

## METHOD OF MANUFACTURING MINERAL WOOL PRODUCT

Filed May 29, 1940



**INVENTOR**  
HAROLD T. COSS.  
WILLIAM M. MACALPINE.  
HERSCHEL V. SWINDELL.  
by *Virgil C. Kline*  
**ATTORNEY**

## UNITED STATES PATENT OFFICE

2,305,516

METHOD OF MANUFACTURING MINERAL  
WOOL PRODUCT

Harold T. Coss, William M. MacAlpine, and Herschel V. Swindell, Somerville, N. J., assignors to Johns-Manville Corporation, New York, N. Y., a corporation of New York

Application May 29, 1940, Serial No. 337,778

10 Claims. (Cl. 154—28)

The present invention is directed to a dry process for the manufacture of mineral wool thermal insulating products of relatively high density and having the desirable properties of insulating materials sold under the registered trademark "Rock Cork," and is a companion case to application Serial No. 336,896, filed May 24, 1940, in the names of Harold T. Coss, William M. MacAlpine, and Louis A. Hawthorne. It will be understood that the term "mineral wool" is employed herein in a generic sense to denote fibres formed from rock, slag, glass, and other conventional raw materials and mixtures thereof.

As has been pointed out in said companion application, the prior known method of manufacturing Rock Cork has been relatively slow and expensive due to the multiplicity of operations involved. Also, certain of these operations have resulted in the mashing or breaking of the fibres, increasing the density and weight of the product to an undesirable extent and decreasing its insulating efficiency; the heterogeneous arrangement of the fibres has reduced the insulating properties of the product; the necessity of molding the product has resulted in a surface crust which must be removed with the resultant loss of material; and the large amount of organic material in the binder has reduced the resistance of the product to combustion.

The instant invention has, as an object, the provision of a method for the manufacture of a product having the desirable characteristics of the present Rock Cork but which overcomes the above-noted disadvantages and in which the operation is continuous from the formation of the fibres to the final packing of the product. More particularly, the instant invention has for an object the provision of such method in which a continuous felt of mineral wool fibres containing a binder disseminated therethrough is subjected to a treatment to compress the felt at and adjacent the surfaces and to set or harden the binder at such locations to form surface layers highly resistant to deformation, and thereafter to a treatment to set the binder in the interior of the felt while the felt is held compressed to a desired thickness.

Our invention will be more fully understood and further objects and advantages thereof will become apparent when reference is made to the more detailed description thereof which is to follow and to the accompanying drawing, in which:

Fig. 1 is a diagrammatic elevational view of a portion of an apparatus employed in the method of the instant invention, and

Fig. 1a is a continuation of the apparatus disclosed in Fig. 1.

Referring now to the drawing, there is diagrammatically shown an apparatus suitable for

carrying out the method of the invention. Conventional portions of the apparatus are not shown in detail as they may take different forms. The apparatus generally comprises a melting furnace 10, which may be a cupola, tank furnace, or the like, of any conventional design. Molten slag, rock, or mixtures thereof, or other conventional raw materials melted in furnace 10, issues therefrom in the form of a stream through orifice 12 and falls into the path of a steam jet 14, which shreds it into a great multiplicity of extremely fine fibres which are carried by the force of the steam jet and in gaseous suspension into blow chamber 16.

15 A binder is forced into the suspension of the fibres by any of the known conventional means for this purpose. Preferably, an atomizing binder jet of a known type, as diagrammatically illustrated at 18, is used. The binder is added in proportions of, say, between 10 to 30% of the weight of the fibres, preferably between 18 and 24%. The mineral wool fibres and the minute binder particles settle in the blow chamber, the binder particles collecting on the fibres.

Binders suitable for use in the instant invention are preferably those referred to in said companion application, wherein the different binder requirements are set out in detail. Briefly stated, it may be said that the binders which have been found most successful are those comprising:

(1) A hard pressure still residue toughened with a softer, blown or refined asphalt, or petroleum tailings. A typical formula is:

|                      | Per cent |
|----------------------|----------|
| Insulating asphalt   | 33.2     |
| Rock Cork asphalt    | 33.2     |
| H. P. asphalt        | 26.6     |
| Chlorinated compound | 7.0      |

35 (2) Gilsonite fluidified with a pressure still residue asphalt, a specific example being:

|                      | Per cent |
|----------------------|----------|
| Gilsonite            | 37.6     |
| Rock Cork asphalt    | 56.5     |
| Chlorinated compound | 6.0      |

40 (3) Thermoplastic resin, for example:

|                      | Per cent |
|----------------------|----------|
| Rosin                | 90.0     |
| Chlorinated compound | 10.0     |

45 In the above-referred-to formulae, the insulating asphalt comprises, for example, a pressure still residue of approximately 214° F. melt point and 1.0 penetration at 77° F. Rock Cork asphalt is an asphalt having a melt point of from 190—205° F. and a penetration of less than 3 at 77° F. H. P. asphalt is a fairly hard, rubbery asphalt having a melt point of 210—220°

F. and a penetration of 5-9 at 77° F. Gilsonite is a natural asphalt having a melt point of 270-325° F. and 0 penetration at 77° F. The chlorinated compound is a chlorinated aromatic or cyclic hydrocarbon with a minimum chlorine content of 45% and is inclined as a fireproofing ingredient. The penetrations and melt points referred to are those determined by standard A. S. T. M. tests. The rosin may be gum or wood rosin, limed rosin, an ester gum, or the like.

The blow chamber 16, which receives the suspension of fibres and binder, has a bottom wall comprising a continuously moving endless belt or conveyor 20 traveling in the direction indicated by the arrow, on which the fibres settle in felted relationship with the binder particles disseminated substantially uniformly throughout the felt. Suitably, the belt may be of a foraminous nature and a suction device provided therebelow as diagrammatically indicated at 22 to aid in securing uniform density of fibre deposit throughout the width of the blow chamber.

The felted mass of fibres is carried from the blow chamber by conveyor 20 and preferably compacted to a slight extent to form a relatively thick blanket 23 by press roll 24 located at the exit end of the blow chamber. Preferably, the rate of movement of conveyor 20 is correlated to the rate of deposition of the fibres to insure uniformity in density of the product as by means of a weighing scale 29 over which the felt passes. Weighing scale 28 is operatively connected to the drive of conveyor 20 by any suitable means (not shown) whereby increase in the weight of the blanket increases the speed of movement of the conveyor and vice versa.

The felted blanket with the binder disseminated therethrough is heated to a temperature sufficient to plasticize the binder. This may be accomplished by an oven 34 including foraminous conveyor belts 28 which carry the felt through the oven, the belts being driven by suitable pulleys 30 in the direction indicated by the arrows. The upper conveyor belt is suitably made vertically adjustable as by means of the mechanism diagrammatically illustrated at 32 and in the operation of the device the belts are so spaced that the blanket is only slightly compressed as it passes therebetween. Air at a temperature, say, between 200-300° F., depending upon the melting point of the particular binder employed, is circulated from any suitable air heating means, such as furnace 35, through ducts 36 opening into the oven below the upper reach of the lower conveyor 28, the heated air being forced through the conveyors and the blanket held therebetween.

Alternatively, the plasticizing of the binder may take place in the blow chamber 16. Depending upon the particular type of blow chamber employed, the residual heat in the fibres may be sufficient for this purpose, or if this is not the case, the temperature of the blanket may be raised to that necessary as by providing heating units or introducing heated air into the blow chamber.

In accordance with our present invention, the blanket passes from the oven 34 or directly from the blow chamber, if the binder is plasticized therein, to a device for compressing and densifying the blanket at the surfaces thereof and for hardening the binder in the condensed surface portions. In its preferred form, this device comprises endless belts 40, suitably mounted for travel in the directions indicated by the arrows

5 around drums 42 and 44. The adjacent reaches of the belts are supported to prevent yielding by beams or other supports 41. The upper belt is arranged for adjustment relative to the lower belt by a raising and lowering device 46. The belts, in this instance, preferably comprise thin steel bands continuous the width of the blanket. Within drums 42, supporting the forward ends of the belts, are provided a plurality of heating means 48, such as gas jets, lamps, or the like, whereby the belts are heated above the melting point of the binder. The gap between belts 46 is adjusted to compress the blanket to substantially less than its desired finished thickness.

15 Located between the drums 42 and 44 are a plurality of cold water sprays 56 or other cooling means which serve to quickly chill the belts and, in turn, solidify the binder adjacent the surfaces of the blanket. The blanket passes from between the belts 40 to a second set of belts 50, supported for travel in the directions indicated by the arrows, on drums 52.

20 The upper belt 50, similarly as in the case of the upper belts of the devices previously described, is mounted to be raised and lowered relatively to the lower belt, the gap between the adjacent reaches of the belt being adjusted so as to compress the blanket to its final desired thickness. Also, the adjacent reaches of both belts are supported to prevent yielding of the same under the pressing action as by means 55. Belts 50 may be steel bands, similarly to belts 40, or may be of any other suitable type. Located between the drums 52 are a plurality of cold water sprays 54 or other cooling means which serve to cool the blanket and solidify the binder throughout the interior of the blanket.

25 The blanket, after leaving the belts 50, passes through any suitable cutting and trimming devices where it is subdivided into blocks or sheets of the desired size and is ready for packing and shipment.

30 In the operation of the method for the production of materials, say, of 2" finished thickness, a felted blanket, which may be, say, 12" in thickness as it leaves the blow chamber and containing a binder of any of the types previously referred to in a proportion between 10 and 30% of the weight of the fibres, is warmed to a temperature, say, of 220-250° F. in oven 34 or in the blow chamber 16 to soften or plasticize the binder. The blanket then passes between heated belts 40 where it is compressed to a thickness of, say, 1½" and then immediately surface chilled by the application of the cold water from sprays 48. It has been determined that the belts 40 should be of such length and driven at such speed that chilling takes place for approximately one minute. The hot belts, during the compression of the felt, serve to convert the binder at and adjacent the felt surfaces to a highly plastic state, whereby a greater condensing of the blanket occurs at the surfaces than in the interior. The chilling of the surfaces hardens the binder in these portions whereby they retain their condensed state.

35 The felt, after leaving the belts 40, expands in thickness due to the resiliency of the felted structure and the still plastic state of the binder in its interior, and passes between belts 50 where it is again compressed, this time to preferably the exact final finished thickness, assumed in the instant example to be 2". While between the belts 50 and held to the desired thickness, at least sufficient of the residual heat is removed

through the action of the cold water sprays 54 to harden or set the binder in the interior of the felt, and preferably, the felt is completely cooled.

The product made as described above has the fibres lying in a plane substantially parallel to the major surfaces whereby the product exhibits increased insulating efficiency as compared to a product in which the fibres are in a heterogeneous arrangement. Also, the modulus of rupture is much higher. The heating of the surface of the blankets between the hot belts 40 and immediate chilling provides the blanket with hard, high density, distortion resisting surfaces, and with a porous interior of substantially less but uniform density.

Having thus described our invention in rather full detail, it will be understood that these details need not be strictly adhered to, but that various changes and modifications will suggest themselves to one skilled in the art, all falling within the scope of the invention as defined by the subjoined claims.

What we claim is:

1. The method comprising forming a suspension of mineral wool fibres and a thermoplastic binder, depositing said fibres to form a felt of substantially uniform density with the binder disseminated therethrough, heating the felt to soften the binder throughout the felt, compressing the felt to a thickness substantially less than the finished thickness while applying heat thereto, hardening the binder in the surface portions of the felt while the felt is under compression, freeing the felt for expansion to a desired finished thickness, and hardening the binder throughout while maintaining the felt at said finished thickness.

2. The method comprising forming a suspension of mineral wool fibres and a thermoplastic binder with the binder disseminated throughout the felt and in a proportion of the order of 10 to 30% by weight of the fibres, plasticizing the binder, compressing the felt to a thickness substantially less than the desired finished thickness, cooling the surfaces of the felt while the same is under compression, freeing the felt for expansion to the desired finished thickness, and cooling the felt throughout while maintaining the same at said finished thickness.

3. The method comprising forming a suspension of mineral wool fibres and a thermoplastic binder, depositing said fibres to form a felt of substantially uniform density with the binder disseminated throughout the felt and in a proportion of the order of 10 to 30% by weight of the fibres, heating the felt to soften the binder, compressing the felt to a thickness substantially less than the desired finished thickness while applying surface heat thereto, cooling the surfaces of the felt while compressed to said thickness, freeing the felt for expansion to the desired finished thickness, and further cooling the felt while maintained at said finished thickness.

4. The method comprising forming a felt from an air suspension of mineral wool fibres and a thermoplastic binder with the binder disseminated throughout the felt and in a proportion of the order of 10 to 30% by weight of the fibres and in a plastic condition, compressing the felt while said binder is plastic to a thickness substantially less than the desired finished thickness, chilling the surfaces of the felt while the felt is maintained at said thickness, freeing the felt for expansion to the desired finished thick-

ness, and cooling the felt while maintained at said finished thickness.

5. The method comprising forming a felt from an air suspension of mineral wool fibres and a thermoplastic binder with the binder disseminated throughout the felt and in a proportion of the order of 10 to 30% by weight of the fibres, slightly compressing the felt, heating the felt to soften the binder, compressing the felt to a thickness substantially less than the desired finished thickness while applying surface heat thereto, chilling the surfaces of the felt while the felt is maintained at said thickness, freeing the felt for expansion to the desired finished thickness, and cooling the felt while maintained at said finished thickness.

6. The method for the manufacture of felted mineral wool products comprising forming an air suspension of newly formed mineral wool fibres 20 and a thermoplastic binder with the binder present in a proportion of the order of 10 to 30% by weight of the fibres, felting said fibres in a blow chamber with the binder substantially uniformly disseminated throughout the felt, heating the felt in the blow chamber to soften the binder, compressing the felt between heated members to a thickness substantially less than the desired finished thickness, chilling the surfaces of the felt while the felt is maintained at said thickness, 30 freeing the felt for expansion to the desired finished thickness, and cooling the felt while maintained at said finished thickness.

7. The method including forming a suspension of mineral wool fibres and a binder, said binder comprising bitumen and a fireproofing ingredient, with the binder present in a proportion of the order of 10 to 30% by weight of the fibres, depositing said fibres to form a felt of substantially uniform density with the binder disseminated therethrough, compressing the felt to a thickness substantially less than the desired finished thickness while applying surface heat thereto, surface chilling the felt while the felt is maintained at said thickness, freeing the felt for expansion to the desired finished thickness, and cooling the felt while maintaining the felt at said finished thickness.

8. The method including forming a suspension of mineral wool fibres and a binder, said binder comprising a hard pressure still petroleum residue, a softer bituminous material, and a fireproofing ingredient, with the binder present in a proportion of the order of 10 to 30% by weight of the fibres, depositing said fibres to form a felt of substantially uniform density with the binder disseminated therethrough, compressing the felt to a thickness substantially less than the desired finished thickness while applying surface heat thereto, surface chilling the felt while the felt is maintained at said thickness, freeing the felt for expansion to the desired finished thickness, and cooling the felt while maintaining the felt at said finished thickness.

9. The method including forming a suspension of mineral wool fibres and a binder, said binder comprising gilsonite fluidified with a pressure still residue asphalt and a fireproofing ingredient with the binder present in a proportion of the order of 10 to 30% by weight of the fibres, depositing said fibres to form a felt of substantially uniform density with the binder disseminated therethrough, compressing the felt to a thickness substantially less than the desired finished thickness, surface chilling the felt while the felt is maintained at

said thickness, freeing the felt for expansion to the desired finished thickness, and cooling the felt while maintaining the felt at said finished thickness.

10. The method comprising forming a felt from an air suspension of mineral wool fibres and a binder, said binder comprising a thermoplastic resin and a fireproofing ingredient with the binder present in a proportion of the order of 10 to 30% by weight of the fibres, depositing said fibres to form a felt of substantially uniform density

5 with the binder disseminated therethrough, compressing the felt to a thickness substantially less than the desired finished thickness while applying surface heat thereto, surface chilling the felt while the felt is maintained at said thickness, freeing the felt for expansion to the desired finished thickness, and cooling the felt while maintaining the felt at said finished thickness.

HAROLD T. COSS.  
WILLIAM M. MACALPINE.  
HERSCHEL V. SWINDELL.